

Patented June 5, 1923.

## UNITED STATES PATENT OFFICE.

ROYER LUCKENBACH, OF BROOKLYN, NEW YORK, ASSIGNOR TO LUCKENBACH PROCESSES, INC., OF SAN FRANCISCO, CALIFORNIA, A CORPORATION OF NEVADA.

## COMPOSITION OF MATTER.

No Drawing.

Application filed February 7, 1920. Serial No. 357,043.

*To all whom it may concern:*

Be it known that I, ROYER LUCKENBACH, a citizen of the United States, and a resident of the borough of Brooklyn, county of 5 Kings, and State of New York, have invented a certain new and useful Composition of Matter, of which the following is a specification.

The invention relates to a composition of 10 matter capable of use in the concentration of ores by flotation, and has for its objects the production of a cheap and efficient mineral gathering and frothing material which may be made up in concentrated form for 15 shipment, which may be introduced directly into the pulp in the flotation apparatus, which will produce a voluminous, viscid and stable froth capable of supporting a maximum amount of mineral, and which may be 20 easily separated from the concentrate and recovered.

These and further objects will more fully appear in the following specification and claims.

25 The present invention is based on the discovery that certain phenols, or hydrobenzenes have powerful mineral selective and gangue repellent properties, and that when combined with a solid pyrogenous bituminous material, such, for example, as a 30 vegetable pitch, will dissolve the latter, and this solution, when treated with an alkaline frothing agent, will adhere to mineral particles and also produce bubbles in the pulp, 35 which bubbles will attach themselves to the coated particles and raise them to the surface of the pulp.

The phenol-bitumin solution, which may be termed a bituminol, is water repellent to a 40 high degree, is in a colloidal condition and will have a high preferential affinity for the non-wettable mineral particles in the pulp, and will repel the wettable gangue particles.

The extremely fine division of the solid 45 or colloidal particles of the bituminol will be conducive to economy of material in that each atom, as it were, of the bituminol will be attracted and attach itself to a mineral particle, and will attract or be attracted by 50 the bubbles and rise with them to the surface.

The preferred materials for use in carrying out the process of the invention are rosin pitch, carbolic acid, and an alcoholic

alkali, or acetone, or both. The pitch, in 55 pulverized condition, is dissolved in carbolic acid until a thick, dark brown liquid results. This liquid is waterproof and will float on water in the form of a film. The thick bitumin-phenol is thinned to the consistency 60 of thin syrup by the addition of an aliphatic compound which may or may not be rendered alkaline. If an alkaline aliphatic compound be used, an alkali, such as caustic soda, may be dissolved in alcohol or acetone 65 and one or both may be employed.

The alkaline alcohol when used may be compounded by dissolving 5 grams of caustic soda or of caustic potash in 1 liter, more or less, of alcohol either ethyl, methyl or a 70 mixture of the two. The alkaline acetone may be made by dissolving 5 grams of caustic soda or potash in about 1 liter of acetone.

As an example of proportions in the reagent, 5 grams of pitch may be dissolved 75 with stirring in 20 cc. of carbolic acid and to the solution may be added 5 cc. of alkaline alcohol and 5 cc. of alkaline acetone, and to the mixture is added approximately 1 liter of warm water. This forms a stock solution 80 which may be added to the pulp in proper proportions to be determined by the character of the ore.

Instead of equal parts of alkaline alcohol and alkaline acetone, 10 cc. of either of those 85 solutions may be employed in the stock solution.

The reagent may be made up for shipment in concentrated form by omitting the water, which may be added on the job. The 90 water in the stock solution is not necessary, but is employed in order that the small proportion of reagent necessary to effect flotation may be more easily measured. If a larger quantity of water be employed in the 95 stock solution the reagent will necessarily be weaker and may be more roughly proportioned to the water of the pulp, or to the ore, than if the stock solution were more concentrated.

100 It has been found that the process may be successfully carried out by using from 2 to 10 cc. of the stock solution wherein 1 liter of water was employed, in 4 liters of pulp water.

105 It is to be understood that the alkaline solution may be greatly concentrated whereby much smaller proportions may be used in

the stock solution. A 10% alkaline solution in water may be made by heating on a water bath.

Instead of using an alcoholic potash in 5 the stock solution, alcohol alone, in approximately the same proportions may be employed, and when so compounded the solution will have an acid reaction.

The bitumin-phenol mixture possesses 10 gathering and frothing properties and may be utilized in the process without the addition of other materials, but when so used it would, because of its water repellent qualities, be necessary to beat it into the water 15 before the pulp is formed or placed in the flotation apparatus, as is the oil in the prior processes.

The addition of the alcohol or acetone either alkalized or not, is for the purpose of 20 emulsifying the mixture whereby the latter will mix with the water of the pulp without previous treatment.

While vegetable pitch is the preferred active material it is to be understood that rosin 25 or other resinous materials may be employed in approximately the same proportions.

The stock solution may be introduced directly into the flotation apparatus without preliminary mixing with the water of which 30 the pulp is to be formed thus reducing operating expenses.

Rosin pitch, the preferred active gathering material, while a rosin derivative is not rosin, nor is it a resin. It is one of the residues of the distillation of rosin (colophony). 35 It is possible that distillation of other resinous substances such as wood, tar, copal, lac, etc. may produce rosin pitch.

It has been found that when operating in 40 certain ores, the mineral gathering and frothing properties may be enhanced by the addition of a small quantity of ordinary glue or gelatin to the mixture. The glue or gelatin is preferably dissolved before it is added to the mixture. It has been found that by dissolving approximately 1 oz. of glue or a like amount of gelatin in 1 quart of water a solution suitable for use in the flotation process may be secured. When the glue 45 water is employed, the alkalized alcohol and acetone may be omitted, or the glue water may be used in addition to the alkaline aliphatic compound.

As a test, a mixture of 5 grams of pitch 55 dissolved in 20 cc. of carbolic acid, and to this mixture was added 40 cc. of the glue water described above. Of the complete mixture 5 cc. was added to about 3 quarts of tap water. To this last mentioned mixture 60 was added 50 gr. of a New Mexico chalcopyrite copper ore which assayed 2.14% cu., to form a pulp.

The pulp was placed in a Case laboratory

flotation machine and a run of 15 minutes was made. The result of the test run was 65 Concentrates 17 grams having a mineral content of 5.57% cu.

Tails 33 grams having a mineral content of 0.29% cu. Extraction 88.5% cu.

The composition of matter described 70 above, while it is particularly useful as a frothing and mineral gathering reagent in the concentration of ore by flotation, may be used for other purposes, such, for example, as a disinfectant. 75

In accordance with the provisions of the patent statutes I have described the principle of my invention, together with the apparatus which I now consider to represent the best embodiment thereof, but I desire to 80 have it understood that the apparatus shown is merely illustrative, and that the invention may be carried out in other ways.

The invention having been described, what is claimed and desired to be secured by Let- 85 ters Patent is:—

1. A composition of matter, comprising a pyrogeneous bitumin, the reaction product of a phenol and an alkali, and the reaction product of acetone and an alkali. 90

2. A composition of matter, comprising a pyrogeneous bitumin, the reaction product of a phenol and an alkali and gelatine. 95

3. A composition of matter, comprising a pyrogeneous bitumin, the reaction product of a phenol and an alkali and glue. 100

4. A composition of matter, comprising a pyrogeneous bitumin, the reaction product of carbolic acid and an alkali and gelatine. 105

5. A composition of matter, comprising a pyrogeneous bitumin, the reaction product of carbolic acid and an alkali and glue. 110

6. A composition of matter, comprising the reaction product of a pyrogeneous bitumin, a phenol and an alkali, and the reaction product of acetone, an alkali and gelatine. 115

7. A composition of matter, comprising the reaction product of a pyrogeneous bitumin, a phenol and an alkali, and the reaction product of acetone, an alkali and glue. 120

8. A composition of matter, comprising the reaction product of a pyrogeneous bitumin, carbolic acid and an alkali, and the reaction product of acetone, an alkali and gelatine. 125

9. A composition of matter, comprising the reaction product of a pyrogeneous bitumin, carbolic acid and an alkali; and the reaction product of acetone, an alkali and glue. 130

This specification signed and witnessed this sixth day of February, 1920.

ROYER LUCKENBACH.

Witnesses:

A. E. RENTON,  
H. LE BERTHON.